

July 31, 1928.

1,679,284

J. WESTLY

PROCESS FOR PRODUCTION OF SELF BAKING ELECTRODES

Filed Jan. 5, 1925



FIG. 1



FIG. 2.

By

*Jens Westly*  
Inventor

*Horsley & Cole*  
Attorney

## UNITED STATES PATENT OFFICE.

JENS WESTLY, OF CHRISTIANSAND, NORWAY, ASSIGNOR TO DET NORSKE AKTIESEL-SKAB FOR ELEKTROKEMISK INDUSTRI OF NORWAY, OF OSLO, NORWAY.

## PROCESS FOR PRODUCTION OF SELF-BAKING ELECTRODES.

Application filed January 5, 1925, Serial No. 712, and in Norway January 17, 1924.

The present application relates to selfbaking electrodes provided with metallic mantles, that is electrodes which are baked in the furnace in which they are used and the object of the invention is a process which makes it possible to avoid introduction of detrimental material from the mantle into the furnace. Such selfbaking electrodes are described in U. S. Patent No. 1,440,724 wherein is stated that one of the functions of the mantle is to transmit the current to the electrode. For that purpose it is often provided with internal ribs or extensions projecting into the electrode mass and facilitating the passage of the current, as these ribs maintain an excellent contact with the mass. Generally both the mantle and the ribs are made of iron and the ribs form a part of the plate from which the mantle is made. The iron melts during the process and enters into the product of the furnace. In special cases the mantle may also be made of other metals, as for instance copper or aluminium. These metals, however, have the drawback that their melting point is considerably lower than that of iron (respectively 150° C. and 660° C.). This drawback is especially noticeable with aluminium, whose melting point is so low that the electrode at that temperature is not yet so well baked that it has even approximately reached its normal electric conductivity. If both mantle and ribs are made of aluminium there will be a greater loss of voltage in the electrode than that normally found when employing iron. I have, however, found that the loss of voltage may be reduced to a considerable extent by making the ribs of comparatively great thickness. They will then allow the electric current to pass through them without being heated to any considerable extent and they will not melt until the surrounding mass has reached a temperature corresponding to their melting point. The ribs may be arranged horizontally or vertically or at any angle with horizontal plane. Further they may be partly horizontal or vertical and partly inclined. A special advantage is obtained if the internal ribs slope downwardly into the electrode mass.

If the metal of the ribs melts it will then not run out of the electrode, but will remain in a pocket in the electrode mass and maintain the connection with the non-molten part

of the mantle. In this way it is possible to effect passage of the current from metal to electrode at temperatures ranging above the melting point of the aluminium and thus supply the current to a better baked electrode mass. Such a construction of ribs is illustrated in the accompanying drawing forming part of this application.

Fig. 1 shows a longitudinal section of an electrode. 3 is the mantle, 4 horizontal internal ribs, 5 inclined internal ribs, which for the purpose of simplicity are shown in one half of the same electrode.

Fig. 2 is a cross section of the same electrode the numerals indicating the same parts as in Fig. 1.

Another modification of my invention consists in reducing the size of the ribs so much that the amount of metal which passes into the furnace on account of the ribs is unimportant as compared with the amount of the product and in such cases the ribs may be made of iron or other material detrimental to the product even if this cannot be permitted in the furnace in larger amounts. This especially applies to furnaces for the production of aluminium. The mantle which is allowed to pass into the bath should of course in such cases not be made of iron, but of a non-detrimental metal such as aluminium and care should then be taken to supply the electric current to the ribs in a safe manner; for instance by means of a clamping arrangement attached to the mantle or to external prolongations of the ribs as described and claimed in my copending application Serial No. 711.

It is of course advisable in the present case to reduce the size of the iron ribs to the minimum possible in order to introduce the least possible amount of the detrimental metal into the furnace. This may be effected by placing the electrode holder as far as possible on baked electrode carbon whereby as much as possible of the current will pass directly over to the electrode under the holder without passing through the ribs. In practice it has in this way been possible to reduce the amount of iron in the ribs so much that the aluminium produced only takes up 0.05-0.1% iron from the ribs.

The amount of iron may be still further reduced if an iron-aluminium alloy is employed in the ribs. Such an alloy with 10% iron melts at about 850° C., that is about

200° C. higher than pure aluminium. The alloy is therefore better adapted for use as rib material than aluminium. It is, however, difficult to roll for which reason it will be preferable to make the ribs by casting.

What I claim as new and desire to secure by Letters Patent of the United States is:

- 5 1. A selfbaking electrode having a mantle of one composition, non-detrimental to the process in connection with which the electrode is being used, and internally projecting ribs of another composition attached to said mantle.
- 10 2. A selfbaking electrode having a mantle of one composition, non-detrimental to the process in connection with which the electrode is being used, and internal ribs composed of a comparatively difficultly fusible metal and attached to said mantle.
- 15 3. A selfbaking electrode having a mantle of one composition, non-detrimental to the process in connection with which the electrode is being used, and internal ribs composed of a comparatively difficultly fusible metal attached to said mantle in combination with an electrode holder attached to a baked part of the electrode.
- 20 4. A selfbaking electrode having an aluminum mantle and internal ribs composed of a comparatively difficultly fusible metal attached thereto.

5. A selfbaking electrode having an aluminum mantle and internal ribs of difficultly fusible metal attached thereto, said ribs being of such small size that they will not 35 introduce a detrimental amount of such metal into the furnace product.

6. A selfbaking electrode having an aluminum mantle and internal aluminum ribs attached thereto, said ribs being of such dimensions as to avoid any considerable heating due to the passage of electric current.

7. A selfbaking electrode having an aluminum mantle and internal aluminum ribs attached thereto, said ribs being of such dimensions as to avoid any considerable heating by the electric current passing therethrough, said ribs being disposed at an angle with the horizontal plane.

8. A selfbaking electrode having an aluminum mantle and internal aluminum ribs attached thereto, said ribs being of such dimensions as to avoid any considerable heating by the electric current passing therethrough, said ribs sloping downwardly into 55 the electrode.

9. A self-baking electrode having an aluminum mantle, and internally projecting ribs of another composition attached to said mantle.

JENS WESTLY.